

# UNITED STATES PATENT OFFICE.

W. E. TASCOTT, OF CLEVELAND, OHIO.

## IMPROVED PAINT-OIL COMPOUND.

Specification forming part of Letters Patent No. 91,578, dated June 22, 1869.

*To all whom it may concern:*

Be it known that I, WILLIAM E. TASCOTT, of Cleveland, Cuyahoga county, Ohio, have invented or discovered a certain Improved Compound for Oil, to be used in the preparation and application of pigments, of which the following is a specification:

This paint-oil aforesaid is composed of rosin, benzine, glue, india-rubber, oxide of manganese, and linseed-oil, which are compounded as follows: I first take the rosin and melt it with glue and water, after which benzine is poured in and stirred up with the first preparation. A compound of india-rubber and linseed-oil is next introduced, then a compound of the oxide of manganese and linseed-oil. The whole mass is then agitated until the ingredients are intimately combined. The proportion of this compound is as follows, viz: I first take fifteen pounds of rosin, one-quarter pound of glue, and two pounds of water, and when combined by stirring over a slow fire in a suitable vessel, it is then withdrawn from the fire, to prevent any accident,

and then three gallons of benzine are added. Next, the preparation of india-rubber and linseed-oil, which is composed of one-quarter pound of india-rubber and one gallon of linseed-oil, which are intimately combined before being mixed in. Then follows the compound of oil and manganese, which is composed of one gallon of oil to half a pound of manganese, which is combined with all the other ingredients and thoroughly stirred up until the entire mass forms an intimate compound. The relative proportions of the several ingredients composing this compound may be used according to the purpose for which the paint may be used, without changing the essential character of my improvements in paint-oil.

What I claim as my improvement, and desire to secure by Letters Patent, is—

The compound for paint-oil, when composed of ingredients substantially as set forth.

W. E. TASCOTT.

Witnesses:

E. E. WAITE,  
W. H. BURRIDGE.